

Nov. 8, 1927.

1,648,471

N. M. AUSTIN

CASTING

Original Filed March 5, 1923

*Fig. 1.*



*Fig. 3.*



*Fig. 2.*



*Fig. 4.*



INVENTOR

Ned M. Austin  
By George, Stebbins & Berndt  
His Atty's

## UNITED STATES PATENT OFFICE.

NED M. AUSTIN, OF CANTON, OHIO, ASSIGNOR TO UNITED ENGINEERING & FOUNDRY COMPANY, OF PITTSBURGH, PENNSYLVANIA, A CORPORATION OF PENNSYLVANIA.

## CASTING.

Original application filed March 5, 1923, Serial No. 622,841. Divided and this application filed January 10, 1925. Serial No. 1,523.

The present invention relates to the art of molding, and more particularly to castings; the present application being a division of my copending application, Serial No. 5 622,841, filed March 5, 1923 and issued as Patent No. 1,544,544 dated July 7, 1925.

In making certain types of castings, particularly cast rolls, it has heretofore been the practice, in order to obtain the desired 10 depth of chill, to employ a composition of metal having the property of freezing quickly. The quick freezing, however, does not allow sufficient time for the graphite to separate out enough to give a solid gray interior to the casting. The quick freezing 15 also has a tendency to set up casting strains which, when a casting is broken, show in the form of radial streaks from the surface toward the center.

20 By the present invention, I propose to overcome the above mentioned and other disadvantages of the prior practice, by effecting a change in the chemical and physical interior structure of a casting after the 25 molten metal has been poured into the mold, and preferably, after the superficial portion of the molten metal has cooled and solidified to form an outer shell. This change is produced by causing the diffusion 30 into the interior of the molten metal of a different metal or material. The invention is of particular importance in connection with the casting of rolls, it being desirable, for example, to lower the melting point of 35 the metal of which the interior of the casting is composed in order that this portion of the casting will not cool too quickly.

Two slightly different methods for practicing my invention are illustrated in the 40 accompanying drawings, in which:

Figures 1 and 2 are similar vertical sectional views of a mold illustrating one method of carrying my invention into effect;

45 Figure 3 is a view similar to Figures 1 and 2, illustrating a slightly modified method; and

Figure 4 is a sectional view of a roll casting made in accordance with my invention.

50 Referring to the drawings, A represents an ordinary sand mold, which may have one or more mold cavities, for casting rolls. This mold has the usual pouring basin 1, strainer core 2, and the vertical and hori-

zontal passages 3 and 4, constituting the 55 gate, for introducing the molten material into the mold, and the riser vents 5. While I have shown a mold for casting rolls, it will be understood that my invention is not limited to rolls, but is applicable to castings 60 generally, irrespective of shape or intended use.

In accordance with the method illustrated in Figures 1 and 2, a pipe 6 is introduced into the mold through a riser vent 5, prior 65 to the pouring of the molten metal into the mold. The lower end of the pipe is closed by a wall of the mold, and the pipe is of some material which will not melt when subjected to the heat of the molten metal 70 surrounding the pipe. The molten metal is now poured into the mold and the superficial portion of the metal surrounding the pipe may be allowed to cool and solidify to form an outer shell. Then the pipe 6 is 75 filled with molten material, which may be another metal, for instance, and the pipe gradually withdrawn from the mold to allow the molten material contained within 80 it to diffuse into the molten metal in the interior of the shell, thereby changing the composition of the casting up to the frozen shell.

In Figure 3, I have illustrated a slight modification of the above described method. 85 According to this method, a bar 7 of different chemical analysis is inserted down through a molten mass of metal in a mold, said bar melting and diffusing into the surrounding metal as in the first method. 90

It will be understood, of course, that in the case of rolls, the object is to obtain extreme hardness in the outer portion of the roll for a considerable depth while giving to the interior of the roll great tensile strength. 95 By the introduction of various metals, in the manner above described, and containing varying proportions of silicon, manganese, carbon, chromium, molybdenum, nickel, copper, cobalt, tungsten, titanium, aluminum and the like, I am enabled to change the internal structure of a roll casting so as to greatly increase the strength of the roll, and I am at the same time enabled to chill to the desired depth. In fact, the present 100 invention enables chilling to greater depths than formerly without weakening the roll.

In Figure 4, I have illustrated a roll cast-

ing made in accordance with either of the methods above described.

I claim:

1. A casting having its outer and interior portions of different compositions, the interior portion consisting of the same material as the outer portion plus additional material diffused thereinto.

2. A casting having a relatively hard chilled outer portion and an interior portion of relatively high tensile strength, the interior portion consisting of the same material as the outer portion, plus additional material diffused thereinto.

3. A casting having a chilled outer portion and a solid gray interior portion of a different composition from said outer portion but formed in part of the same material as the outer portion of the casting.

4. A casting roll for rolling mills having a chilled outer portion and a solid gray interior portion of a different composition from said outer portion and formed of the same material as the outer portion but having alloying material diffused therethrough.

In testimony whereof I have hereunto set my hand.

NED M. AUSTIN.